

## UNITED STATES PATENT OFFICE

2,150,353

## REFINING OF WHITE METALS

Gustave E. Behr, New York, N. Y., assignor to  
 National Lead Company, New York, N. Y., a  
 corporation of New Jersey

No Drawing. Application January 4, 1938,  
 Serial No. 183,319

8 Claims. (Cl. 75—63)

This invention relates to the elimination of impurity such as aluminum from metal and alloys, being usually present in only fractional percentages as, for example, in lead or lead tin alloys, such as solder or so-called white metals. Even as little as .00025 per cent aluminum in solder is definitely objectionable.

Heretofore the aluminum has been cleared by stirring sal ammoniac or sulphur into the metal, but the use of these clearing agents and all others of which I am aware, produces ill-smelling smoke and fume, which is not only unpleasant to the workmen but pollutes the atmosphere in the locality where the operation is carried on and is particularly objectionable on that account.

The object is to provide means for clearing the metal of the contaminating aluminum with all the efficiency and convenience of the present practice, but without producing the objectionable fume and smoke.

To this end, the invention consists, in its preferred form, of a compound containing the following ingredients in substantially the proportions indicated:

|                                          | Per cent |
|------------------------------------------|----------|
| 25 Na <sub>2</sub> CO <sub>3</sub> ----- | 42.5     |
| NaCl-----                                | 17       |
| KCl-----                                 | 25.5     |
| NaOH-----                                | 15       |

30 This mixture melts at about 590° C. and is commonly used by placing it on the metal to be cleared before beginning the melting process, and in sufficient quantity to cover the surface when melted. Being a relatively poor conductor 35 of heat, the mixture forms a heat conserving cover enabling the metal to be quickly melted. When the temperature reaches 593° C. or more, a mechanical stirrer is set on the kettle rim and started. In about 15 minutes the metal, when 40 uncovered, will give the signs of aluminum-free metal. The stirrer is then stopped and the melted salt mixture skimmed off. The addition of a pinch of sulfur will then finish the metal so that it will pour a perfect solder bar. If the solder is poured immediately after 45 skimming, the bars will have a fogged appearance. To clear this, sal-ammoniac or rosin in very small amounts can be used but the amount of either sulfur, sal-ammoniac or rosin used for 50 this is insignificant from the fume-producing point of view. The last detectable trace of aluminum can be thus eliminated from the metal without producing objectionable fumes. Elaborate ventilation equipment is no longer needed

and there is no pollution of the atmosphere. While the invention has been devised more particularly for removing aluminum, it is found also useful for removing zinc which responds similarly to aluminum.

The new compound has the property of eliminating the impurity without affecting or removing any appreciable amount of tin. It is highly selective in its action notwithstanding that the amount of tin present may be, in an ordinary case, some 200,000 times the amount of aluminum. It can be used a number of times before becoming exhausted and longer if replenished from time to time to make up for losses and the gradual thickening that is due to the impurity taken up. When the mixture has thickened as much as consistent with good operation, a separation of thick and thin salts can be made in a simple manner. The used salts are remelted in a kettle. Three layers will result. The top layer is thin-melting salts and is ladled off for further use. The middle layer consists of thickened used-upsalts and this is ladled out and reserved for recovery if it has sufficient value. The bottom layer is clean metal from the kettle inevitably held in the salts as the result of the vigorous stirring.

The principal aluminum-eliminating agent is the sodium carbonate which like other alkali-metal carbonates, as I have discovered, is effective by itself for clearing out small traces of aluminum, doing it selectively without affecting the tin and the invention includes such use, although sodium carbonate is best employed in conjunction with the other components in the formula above given, or their equivalents having the function of lowering the melting point and therefore the temperature of the treatment, so that the kettle, usually iron, does not need to be so highly heated and so that the loss by drossing, always greater with high temperatures, is reduced. Various substances or combinations of substances may be used for this purpose, provided they are inert to the kettle contents, except the aluminum, and provided also they are non-fume-producing.

For example, a mixture of sodium or other alkali-metal carbonate 50%, sodium chloride 20%, and potassium chloride 30%, makes a compound melting at about 582° C., which is practical for the treatment and also fumeless. The maximum permissible melting point is controlled by the nature of the kettle and is assumed to be about 650° C. Any inert and fumeless compound

of salts producing a lower eutectic temperature will be found suitable.

5 Alkali hydroxides, although fumeless, would not ordinarily be selected when tin is present, because they are known to have a rapid action on that metal in metallic alloys, but I have found that within limits the presence of such hydroxides not only contributes to a lower melting point of the compound, but also accelerates its action 10 and without any noticeable effect on the tin. This may be the result either of a critical degree of dilution of the caustic by the other components as diluents, or of a certain inhibiting effect exercised by sodium carbonate. In any event, 15 I have found that this effect occurs in the compound containing up to 15% of sodium hydroxide and this substance is accordingly used in the preferred formula above given. The use of more than this proportion is possible, but at the risk 20 of tin loss.

It will be recognized that the proportions above given as preferred are approximately representative of a quaternary eutectic. Deviations therefrom are permissible, but only so long 25 as the melting point of the compound is kept within the practical limit of 650° C.

I claim:

30 1. The process of removing aluminum impurity from tinny metals which consists in selectively removing the aluminum, with reference to the tin, by treating the molten, tinny metal with a molten alkali metal carbonate.

35 2. The process of removing aluminum impurity from tinny metals which comprises selectively removing the aluminum, with reference to

the tin, by treating the molten tinny metal with a molten mixture of alkali metal carbonate and a non-fuming melting-point depressant.

3. The process of removing aluminum impurity from lead-tin alloys which comprises selectively removing the aluminum, with reference to the tin, by treating the molten alloy metal with a molten mixture of an alkali carbonate and alkali-metal chloride in substantially eutectic proportions. 5

4. The process of removing aluminum impurity from lead-tin alloys which comprises selectively removing the aluminum, with reference to the tin, by treating the molten metal with a mixture of an alkali metal carbonate and an alkali 15 metal hydroxide.

5. The process of claim 4 in which the hydroxide is present in amount not exceeding about 15% of the mixture.

6. The process of claim 4 in which the hydroxide is present in amount not exceeding about 15% and the mixture contains also alkali metal chloride or chlorides. 20

7. As a clearing agent for contamination in lead-tin alloys, a mixture compound of alkali metal carbonate, hydroxide and halide in proportions melting below 650° C., the carbonate predominating. 25

8. As a clearing agent for aluminum contamination in tinny metals, a mixture compound of about 42.5% sodium carbonate, 17% sodium chloride, 25.5% potassium chloride and 15% sodium hydroxide. 30

GUSTAVE E. BEHR. 35